

## UNITED STATES PATENT OFFICE.

CHAD H. HUMPHRIES, OF KOKOMO, INDIANA, ASSIGNEE, BY MESNE ASSIGNMENTS, TO METALS PROTECTION CORPORATION, OF INDIANAPOLIS, INDIANA, A CORPORATION OF INDIANA.

PROCESS OF PRODUCING CORROSION-RESISTING COATING ON IRON AND STEEL AND PRODUCTS.

No Drawing.

Application filed June 5, 1924. Serial No. 718,080.

I have found that by applying a very thin coating of chromium over the coatings of other metals upon iron and steel products having very desirable corrosion resisting properties may be produced, and further that the chromium coating can be produced in such form that further mechanical finishing thereof is unnecessary.

In a copending application in the names of Harrie C. Pierce and Chad H. Humphries, Serial No. 711,256, filed May 25, 1924, (now Patent No. 1,545,196) there is described a method of producing extremely thin continuous and coherent coatings of chromium upon other metals. Such chromium coatings have excellent corrosion preventing properties. Under certain circumstances, however, it is unwise to trust solely to the chromium coating. The present invention therefore relates to the application of multiple coatings of certain metals, the outermost of which coatings is chromium, and to the products so produced.

The invention embraces quite a variety of combinations of coatings among which may be mentioned by way of example the following: chromium on copper on iron or steel; chromium on brass on iron or steel; chromium on copper on cadmium on iron or steel; chromium on copper on zinc on iron or steel; chromium on brass on cadmium on iron or steel; chromium on brass on zinc on iron or steel; chromium on cadmium on iron or steel; chromium on zinc on iron or steel; chromium on nickel on iron or steel.

The coatings may be applied by any suitable electroplating methods but with regard to the chromium coating it is desirable from a commercial standpoint that a process be used which will give a lustrous coating at low current density, otherwise, for instance if a high current density is required or if the coating is not lustrous, some of the value of the composite coating from a commercial standpoint is lost. I therefore prefer to use the process of chromium plating which forms the subject matter of the Pierce and Humphries application Serial No. 711,256, above referred to. Said process consists

generally in electrodepositing chromium at 50 a relatively low current density, say from 14 up to 125 amperes per square foot, but preferably in the neighborhood of 14 to 40 amperes per square foot, from a bath containing essentially chromic acid, ammonium 55 sulfate and hydrated chromic hydroxid dissolved in water at room or slightly elevated temperature, using either inert or chromium anodes.

The bath may be prepared by mixing a 60 solution of chromic acid in water with a solution of the reaction products of chromic sulfate and ammonium hydroxide in water. The quantity of chromic acid used may vary 65 from 80 to 450 grams per liter of the final solution. The chromic sulfate is used in quantity amounting to 1 to 2% of the chromic acid and the ammonium hydroxide preferably in quantity about chemically equivalent to the chromic sulfate. The invention is 70 not limited to the use of the particular bath and process for applying the chromium coating described above. The so-called "Sargent's" solution for which somewhat higher current densities are recommended 75 may be used.

The following examples illustrate the process:

(1) Iron or steel articles, properly prepared mechanically for finish and by ordinary plating room cleaning methods to receive an electrodeposited coating, are plated in a zinc cyanide bath with a coating of zinc approximately .0001 inch or more in thickness, rinsed in water and given an electrodeposited coating of copper or brass from a copper cyanide or standard brass plating bath, subjected to mechanical buffing or to a bright acid dip to give the copper or brass coating a high luster, and then coated with 85 chromium by means of the Pierce and Humphries chromium plating process described above.

(2) Iron or steel articles properly prepared for electroplating and finishing as described in Example 1 are plated with copper in a cyanide copper plating bath alone or in a cyanide copper bath and then in an

acid copper bath to produce the desired thickness of the copper coating and then plated with chromium as described.

The multiple coatings with chromium on the outer surface produced in accordance with this invention give remarkable atmospheric corrosion and acid fume resisting properties to the coated articles. A coating of chromium on copper on zinc on steel with the zinc coating .0001 inch thick and the copper coating .0001 inch or less thick and the chromium coating .00006 inch or less thick by computation, after being subjected to the standard salt spray test for 80 hours showed no evidence of rust streaks or areas, or pin holes, and the original bright luster of the chromium coating was undimmed. For comparison it is noted that standard nickel on steel and nickel on copper on steel platings subjected to the same salt spray test failed in 10 hours, while a nickel on cadmium on steel coating failed in 24 hours. The chromium coated articles not only withstand corrosion longer than the other standard coatings referred to, but have the additional and very important further advantage that they retain their luster and do not become dulled or tarnished.

The chromium coatings should not be of less than a computed thickness of .00006 inch, because with coatings of less than this thickness there is a tendency for the under coatings to show through after standing, there being evidence of chromium absorption.

Of the composite coatings those in which the chromium over-coating is deposited directly upon an under-coating of copper or brass are preferred because chromium coatings upon copper and brass show a greater tendency to be lustrous and the production of a lustrous finish directly obviates the more or less expensive mechanical coloring treatment which otherwise would be necessary in order to produce lustrous finishes. When the copper or brass coating is deposited directly upon the iron or steel it should be made somewhat heavier than when the undercoating of cadmium or zinc is used.

The corrosion resisting properties of the composite coatings of the present invention may be explained in part by the fact that the chromium coatings are very hard and protect the undercoating against abrasion. A further explanation is as follows.

When iron is protected against corrosion by coatings of metals such as cadmium and zinc which are electropositive to iron the protection is given by the preferential oxidation of the coating metal while when coatings of nickel alone or nickel on copper on iron are used, the protective action is due solely to the continuity of the coatings since both copper and nickel are electronegative to iron. In the case of coatings of nickel on

cadmium or zinc on iron the intermediate metal, cadmium or zinc which is electropositive to both the iron and nickel, is very rapidly used up due to electrolytic action in case pin holes or breaks in either the iron or nickel occur. Such conditions do not exist in the coatings of the present invention. For instance in the case of the coating of chromium on copper on cadmium on iron the relationship is as follows. Cadmium is positive to iron, copper is negative to the cadmium and the chromium is electropositive to both the copper with which it is in contact and also to the iron. In the case of chromium on copper on iron, the more electropositive metal is on the outside and not as in the case of nickel on cadmium on iron, sandwiched between two electronegative metals. In the case of chromium on zinc on iron both of the coating metals are electropositive to the iron.

Throughout the specification and in the claims, I mean by an electropositive metal, a metal electropositive to iron, and above iron in the electromotive series, such as zinc, or chromium. By electronegative metals, I mean metals below iron in the electromotive series, such metals being nickel, copper, etc.

There is a discrepancy in the literature with regard to the designation of elements in the electromotive series and for purposes of clarity and consistency, the following table, taken from Mellor's "Modern Organic Chemistry" (1917 edition, page 363) is appended.

|            |           |
|------------|-----------|
| Sodium.    | Cobalt.   |
| Magnesium. | Nickel.   |
| Chromium.  | Tin.      |
| Manganese. | Lead.     |
| Zinc.      | Hydrogen. |
| Cadmium.   | Copper.   |
| Iron.      |           |

The more electropositive metals are at the top of the table. Thus zinc is electropositive to iron whereas copper or nickel is electronegative to iron.

Not all of the elements listed in the Mellor table have been listed herein. The purpose of the table is to show the relative positivity and negativity of the metals towards iron. Thus, chromium on copper on cadmium on iron or steel bears the relation, potentially speaking, of a metal electropositive to iron superposed on an electronegative metal which is in turn superposed on an electropositive metal plated on an iron or steel base.

I claim:

1. Process of protecting iron and steel articles against corrosion which comprises applying to the surfaces thereof an over-coating of chromium on an under-coating of copper.

2. As an article of manufacture a piece of iron or steel having a composite coating com

prising a layer of copper and a superposed layer of chromium.

3. An electroplated article consisting of a steel base, a copper coat electro-deposited thereon, and a chromium coat electro-deposited on the copper.

4. A process of electroplating steel or the like, consisting in first cleaning the surface

to be plated, then electroplating a copper coat thereon, and finally electroplating a <sup>10</sup> chromium coat on the copper coat.

5. The method of protecting steel which consists in coating it with copper and chromium.

In testimony whereof, I affix my signature.

CHAD H. HUMPHRIES.